

Jan. 17, 1950

C. B. LEAPE

2,495,173

NONCRYSTALLINE SYNTHETIC RESIN HOLDER

Filed June 19, 1947

Fig. 1.



Fig. 2.



Fig. 3.



Fig. 4.



WITNESSES:

Robert O'Baird  
Rev. C. Groome

INVENTOR

Charles B. Leape.

BY  
Frederick Shapoe  
ATTORNEY

## UNITED STATES PATENT OFFICE

2,495,173

NONCRYSTALLINE SYNTHETIC RESIN  
HOLDER

Charles B. Leape, Pittsburgh, Pa., assignor to  
Westinghouse Electric Corporation, East Pitts-  
burgh, Pa., a corporation of Pennsylvania

Application June 19, 1947, Serial No. 755,752

2 Claims. (Cl. 250—51)

1

This invention relates to holders for retaining samples of powder gums or the like which are to be subjected to various tests and particularly X-ray diffraction tests.

In performing X-ray diffraction tests, particularly with powders and similar materials that are not in the form of a unitary solid, it is necessary to position the material in such a manner that it is completely bathed in a relatively narrow beam of X-rays. A loose powder cannot be properly tested and it is necessary to unite the powder with some adhesive material to produce a unitary member. The prior art techniques have been found to be quite cumbersome as well as time consuming as well as being unreliable at times. In other cases, it has been impossible to test numerous certain organic materials by conventional procedures due to their reactivity and other properties. While it has been suggested that an envelope might be prepared from a resinous material and the powders or crystals be placed within the envelope and thus tested. However all previously known resins appear to have a characteristic X-ray pattern due to a crystalline structure. This creates an interfering X-ray pattern on testing such a combination. Confusion between the interfering X-ray diffraction pattern of the powder being tested and the resin holder thus arises and misleading results may be reported. This is particularly true with numerous resinous materials that may have a strong pattern or a pattern quite similar to that possessed by the material being analyzed or tested.

The present invention is based on the discovery of a non-crystalline or isotropic resin. This isotropic resin has been found to be eminently suitable for a holder or envelope for samples of powders and the like to be subjected to X-ray diffraction testing.

The object of this invention is to provide a sample holder having substantially no crystalline structure observable on X-ray diffraction tests.

A further object of the invention is to provide an envelope sample holder composed of a poly-ester-amide resin composition having substantially non-crystallinity observable on X-ray diffraction testing.

Other objects and advantages of the invention will in part appear hereinafter and will in part be obvious. For a better understanding of the nature and objects of the invention, reference should be had to the following detailed description and drawing, in which:

Figure 1 is a view in elevation, partly in section, of the preparation of holders;

2

Fig. 2 is a view in elevation, partly in cross section, of a closed end holder;

Fig. 3 is a view in elevation, partly in cross section, of a tube form of holder; and

Fig. 4 is a view in perspective of a holder prepared by sealing the edges of a sheet of resin.

Referring to Fig. 1 of the drawing, there is illustrated an apparatus for producing holders in the form of thin tubes closed at one end from the isotropic and relatively non-crystalline resinous compositions to be disclosed hereinafter. The tank 10 contains the solution 12 of the isotropic resinous composition. A bar 14 containing a number of round ended fingers 16 is located for movement into and out of the composition 12 whereby a film of the composition may be dip-coated on the fingers to a selected depth. A fine capillary bore 18 passing through the center of each of the fingers 16 is connected to a channel 20 which, in turn, is connected by a conduit 22 controlled by valve 24 to a source of compressed air or gas 26.

Upon dipping the fingers 16 one or more times into the composition 12 and drying to evaporate the solvent from the composition, a resinous coating in the form of a closed end holder 28 is present on the tip of each of the fingers 16. The bar 14 with the coated fingers may be subjected to heating by infrared radiation or hung in an oven in order to cure the resin partly or entirely to permit the removal of the resinous holders 28 from the fingers. This is accomplished by opening the valve 24 to admit air from the source 26 into the channel 20 and thence to each of the capillary bores 18 thereby blowing off the holders 28. The separated holders 28 may be cured at a temperature of 150° C. or higher for a few minutes if insufficiently cured previously. The fingers 16 may be initially coated with a film of a suitable parting compound before dipping in the composition 12 to facilitate the easy separation of the resinous holders 28 from the fingers 16. The fingers 16 may be made of metal such as aluminum or copper, or from glass or even certain resinous compositions.

The resinous composition 12 is a unique isotropic polyester-amide type product prepared by reacting a combination of unsaturated and saturated dicarboxylic acids or anhydrides of the unsaturated dicarboxylic acids, polyhydric alcohol and aliphatic diamine. The unsaturated dicarboxylic acid is selected from the group consisting of maleic acid, fumaric acid, maleic anhydride and the monomethyl substitution de-

rivatives for the noncarboxyl hydrogens thereof. Citraconic acid and citraconic anhydride are examples of such monomethyl derivatives. In combination with the unsaturated dibasic acid is a lesser molar amount of saturated aliphatic hydrocarbon dicarboxylic acid, selected from dicarboxylic acids having from 1 to 12 non-carboxyl carbon atoms, and including at least 25 mole-percent of succinic acid. Reacted with the combination of dicarboxylic acids are a diamine selected from the group consisting of ethylene diamine and propylene diamine, and a polyhydric alcohol, the major proportion of which is a glycol. Suitable polyhydric alcohols are ethylene glycol, propylene glycol, diethylene glycol, hexamethylene glycol, glycerol and pentaerythritol.

In producing the resin, the unsaturated dibasic acid and saturated dibasic acid in an amount totaling from 7.2 to 8.8 moles are reacted with the aliphatic diamine and polyhydric alcohol totaling the same number of moles or with a molar excess of up to as much as a third more.

In general, the saturated dicarboxylic acid may be either a single acid or a mixture of several dicarboxylic acids having from 1 to 12 non-carboxyl carbon atoms selected to provide an average of from 2 to  $3\frac{1}{2}$  noncarboxyl carbon atoms per dicarboxylic acid molecule. However, at least 25 mole-percent of the saturated dicarboxylic acid should be succinic acid, since succinic acid appears to be critical in securing satisfactory enamel coatings.

More specifically, exceptionally good synthetic resins are prepared from about 4.25 to 5.9 moles of the unsaturated dicarboxylic acid or anhydride thereof, such as maleic anhydride, and from 2 to 4.8 moles of a saturated dicarboxylic acid of which at least 25 mole-percent is succinic acid. Good results have been obtained with only succinic acid as the saturated dicarboxylic acid. From 2.1 to 2.65 moles of either ethylene diamine or propylene diamine or a mixture of both is combined with from 5 to 6.75 moles of a glycol or a mixture of polyhydric alcohols of which the major proportion is a glycol.

The following example is indicative of a mode of preparation of the synthetic polyester-amide resins of this invention:

*Example I*

|                  | Moles |
|------------------|-------|
| Maleic anhydride | 5.34  |
| Succinic acid    | 1.33  |
| Adipic acid      | 1.33  |
| Ethylene glycol  | 5.6   |
| Ethylene diamine | 2.4   |

were reacted by placing the first four ingredients in a reaction vessel equipped with a thermometer, stirring means, gas inlet tube, an outlet tube for removing water liberated during the reaction, and a dropping funnel. After the four ingredients had been stirred into a uniform mixture, the ethylene diamine was added to the solution slowly from the dropping funnel with rapid stirring. The rate of addition of the ethylene diamine was so adjusted that approximately ten minutes were required to add it to the reaction vessel contents. An exothermic reaction occurred during the addition of the ethylene diamine which caused the temperature to rise from 100° C. to 115° C. After the addition of ethylene diamine was completed, the reaction vessel was heated externally so that the temperature rose slowly. At about 130° C., water vapor was given

off and was swept out by a flow of nitrogen gas admitted to the interior of the reaction vessel through the gas inlet tube. The heat input was so adjusted that, after approximately two to eight hours, a temperature of 150° C. was reached. Good results are secured if a period of six hours is taken to reach 150° C. The rate of rise of temperature was maintained at this rate, or even at a somewhat slower rate, until the reaction product reached a maximum temperature of about 170° C. to 175° C. At this point, the ball and ring temperature of the resinous reaction product was from 45° C. to 90° C. The reaction was then terminated by diluting the resinous reaction product with a solvent in an amount sufficient to produce a composition having about 50% to 60% resin solids. The relatively concentrated resin solution was then cooled rapidly to room temperature.

Various solvents may be employed for dissolving the polyester-amide reaction product to produce a solution thereof. Suitable solvents are diacetone alcohol, cresol, toluene, equal parts of a cresol and ethyl alcohol mixture, equal parts of a cresol and petroleum fraction boiling in a temperature range of from 50° C. to 75° C., and mixtures of cresol with ethyl lactate, solvent naphtha, tetrachloroethane, ethylene dichloride, trichlorbenzene or monochlorotoluene. This list is merely exemplary and not limiting since numerous other organic liquids and various mixtures of organic liquids may be employed as solvents.

The reactants of Example I may be varied from 5 to 5.75 moles of maleic anhydride, from 1.2 to 1.5 moles each of adipic and succinic acids, from 2.1 to 2.65 moles of ethylene diamine and from 5 to 6.75 moles of ethylene glycol, the acids being balanced to produce the same molar total and the diamine and glycol being similarly balanced.

The order of reaction of the ingredients of Example I is not particularly critical. For example, the diamine may be reacted with either of the unsaturated or saturated dibasic acids before combining with the glycol and the other acid. The rate of reaction may be increased or decreased considerably without notably affecting the product. In general, the procedure under Example I gives the best results. Obviously, the end point of the reaction may be modified to suit the intended application of the resins. The reaction may be so conducted as to carry the resins to a more advance state of polymerization, or to a lower degree of polymerization for some applications. In these ways, resins of varying degrees of toughness and flexibility may be secured, thus allowing a broad latitude in meeting various requirements.

*Example II*

|                  | Moles |
|------------------|-------|
| Fumaric acid     | 5.34  |
| Succinic acid    | 1.33  |
| Adipic acid      | 1.33  |
| Ethylene diamine | 2.4   |
| Ethylene glycol  | 5.6   |

The ingredients were reacted as in Example I, the fumaric acid replacing the maleic anhydride in that example. The resinous compositions produced herein have certain highly desirable characteristics. X-ray diffraction studies indicate substantially no crystallinity. Films of this resin have been prepared in various ways and no crystallinity has been found by X-ray diffraction studies. Even

when stretched, no substantial amount of crystallinity or orientation has been found. This indicates a high degree of isotropicity and homogeneity of structure.

Referring to Fig. 2 of the drawing, there is illustrated a greatly enlarged view of one of the holders 28 as prepared in the apparatus of Fig. 1. The holder comprises a relatively uniform internal bore terminated by a closure 30 and has an open end 32 for introducing a powdered or other sample into it. The open end may be sealed if desired after the sample has been introduced.

In Fig. 3 of the drawing, there is illustrated a greatly enlarged view of a different form of a tubular holder 40 having open ends 42. The tubular holder of Fig. 3 is prepared by coating copper wire in the isotropic resinous composition. A suitable diameter for the copper wire is from about 0.25 to 1.0 millimeter. The wire may be much larger or somewhat smaller to suit the size of tubular holder desired. The thickness of the composition on the wire may be approximately 0.010 millimeter after baking in an oven for a few minutes at temperatures of around 350° C.-450° C. to cure the resin to a hard thermoset condition. The wire is then aged in an oven for 36 hours at 150° C. The wire is cut into short lengths and upon jerking these lengths suddenly to elongate the copper about 25% or more, the resinous coating is freed from the copper and can be readily slipped off. Tubes of any suitable length can then be prepared by cutting. The tubes can be filled by tapping the holder against the powdered or crystalline material on a glass plate, inverting and shaking, and repeating to fill the tube up. The ends of the tubes may be sealed with a similar resin or other adhesive material since the ends are not subjected to X-ray beam.

If desired, sheets of the resinous composition may be prepared by flowing a predetermined amount of the resinous composition upon glass plates or upon sheets or blocks of polytetrafluoroethylene and curing them to a thermoset condition whereupon they may be stripped from the base. The sheets may then be cut to selected length and width and, as illustrated in Fig. 4, the edges may be cemented with some of the solution of the resinous composition. In Fig. 4 the holder 50 comprises a sheet 52 with the edges sealed together at 54 with some of the same composition as that from which the sheet 52 is composed. The envelope or holder so prepared may be filled in the usual manner.

It will be apparent that there are numerous other forms of materials that may be prepared from the resinous compositions disclosed herein. Therefore, the above description and drawing are intended only to be exemplary and not exhaustive.

I claim as my invention:

1. A holder suitable for holding samples for X-ray diffraction tests comprising a thin walled cylindrical member having a longitudinal passage

for receiving a material, the walls of the cylindrical member being composed of a substantially non-crystalline resin when observed on X-ray diffraction tests, the resin being composed of the heat cured resinous reaction product of from 4.25 to 5.9 moles of an unsaturated acidic compound selected from the group consisting of maleic acid, fumaric acid, maleic anhydride and the mono-methyl substitution derivatives for the non-carboxyl hydrogen thereof, from 4.8 to 2 moles of a mixture of saturated hydrocarbon aliphatic dicarboxylic acids having an average of from 2 to 3½ non-carboxyl carbon atoms per acid molecule selected from the group consisting of saturated aliphatic dicarboxylic acids having from 1 to 12 non-carboxyl carbon atoms, the saturated dicarboxylic aliphatic acids composed of at least 25 mole-percent of succinic acid, the moles of the acidic ingredients totaling from 7.2 to 8.8, from 2.1 to 2.65 moles of aliphatic hydrocarbon primary diamine, the aliphatic diamine having an average of from 2 to 3 carbon atoms per molecule, and from 5 to 6.75 moles of a mixture of aliphatic polyhydric alcohols having no other reactive groups than the hydroxyl groups, the major proportion of the polyhydric alcohol mixture being glycol, the total moles of aliphatic diamine and polyhydric alcohol substantially equal to at least the moles of the acidic ingredients but not in excess of ½ of the moles of the latter.

2. A holder suitable for holding samples for X-ray diffraction tests comprising a thin walled cylindrical member having a longitudinal passage for receiving a material, the walls of the cylindrical member being composed of a substantially non-crystalline resin when observed on X-ray diffraction tests, the resin being composed of the heat cured resinous reaction product of from 5 to 5.75 moles of maleic anhydride, from 1.2 to 1.5 moles of succinic acid, from 1.2 to 1.5 moles of adipic acid, the three acidic ingredients totaling substantially 8 moles, from 2.1 to 2.65 moles of ethylene diamine and from 5 to 6.75 moles of ethylene glycol, the ethylene diamine and glycol totaling at least 8 moles.

CHARLES B. LEAPE.

#### REFERENCES CITED

50 The following references are of record in the file of this patent:

#### UNITED STATES PATENTS

| Number    | Name                  | Date          |
|-----------|-----------------------|---------------|
| 1,546,349 | Hull et al. _____     | July 14, 1925 |
| 2,048,778 | Brubaker et al. _____ | July 28, 1936 |
| 2,282,827 | Rothrock _____        | May 12, 1942  |
| 2,285,370 | Staelin _____         | June 2, 1942  |
| 2,424,884 | Cook et al. _____     | July 29, 1947 |

#### OTHER REFERENCES

60 Structure of Metals, by C. S. Barrett, published by McGraw-Hill Book Co., New York, 1943, p. 118.